# EUROPEAN PATENT SPECIFICATION

(11) **EP 0 849 013 B1**
(45) Date of publication and mention of the grant of the patent: **11.04.2001**
(21) Application number: 97203563.8
(22) Date of filing: 14.11.1997
(51) Int. Cl.: B21D 26/02

(54) **Advanced forming techniques for superplastic forming**
Verbesserte Formtechnik für superplastische Formung
Technique de formage améliorée pour le formage superplastique

(30) Priority: 21.12.1996 US 773728
(43) Date of publication of application: 24.06.1998
(73) Proprietor: THE BOEING COMPANY, Seattle, Washington 98124-2207 (US)
(72) Inventor: Beal, Joseph D., Auburn, Washington 98001 (US); Takayama, Chris J., Bellevue, Washington 98008 (US)
(74) Representative: Land, Addick Adrianus Gosling

(56) References cited:
- US-A- 4 748 837
- US-A- 4 984 348
- US-A- 5 419 170

## Description

### 1. Field of the invention

The present invention relates to techniques for superplastic forming of parts, and more particularly, for control.

### 2. Background of the invention

Superplastic forming hereinafter (SPF) is a metal forming process used throughout the aerospace industry for manufacturing detailed parts and built-up structures. The design flexibility that is offered by SPF has resulted in substantial cost savings in the fabrication of detail parts and assemblies. Further savings have been apparent in the reduction of weight in aircraft. The prior art SPF process for manufacturing parts consists of several steps. These steps are illustrated in figures 1A to 1D and can be summarized as follows: heating a die to an appropriate temperature for a particular metal alloy; placing a metal sheet, also reffered to as a blank, in the die; closing a lid to the die; applying restraining forces to hold the die and lid together; applying a forming gas pressure to the blank in order to push the blank into the die cavity; completing the time required in the forming cycle; and removing the finished part from the die.

Figure 2 shows a schematic plan view of the die with the lid removed for illustration purposes. The blank or sheet 10 is supported in the regions 12 surrounding the sealed area 14 by the lower die 16, as shown in figure 1A. The double lines 18 outline the seal area, within which a part will be formed. The reason that the material does not thinout uniformly is that once the lid is closed on the SPF die, the periphery of the material is restrained such that the material is not allowed to "draw-in" the material outside of the seal area.

Figure 3 shows a schematic cross section view of a part formed by SPF. The dotted lines show where die part will be cut or trimmed. The run-out is in the die region outside of the net part area. A correctly designed die will optimize the run-out configuration so that thinout is minimized in the part area and maximized in the run-out material.

Figure 4 is a side elevation cross-section illustrating the thinout problem. For example, the part thicknesses at 20 and 22 are very thin, and could potentially be below the thicknesses specified by the Engineering drawing.

US-A-4984348, Cadwell disclosing the state of the art as described in the precharacterising portion of claim 1, refers to the drape forming techniques of SPF. However, the blank associated herewith is subject to undesirable deformation during superplastic forming.

### Summary of the Invention

The invention is defined by the combined features of claim 1. The dependent claims define preferred embodiments of the invention.

### Brief Description of the Drawings

The foregoing aspects and many of the attendant advantages of this invention will become more readily appreciated by reference to the following detailed description, when taken in conjunction with the accompanying drawings, wherein:
**FIGURES 1A** to **1D** are a side elevation cross-section drawing of a prior art SPF in four consecutive modes of operation.
**FIGURE 2** is a plan view of a die with lid removed.
**FIGURE 3** shows a schematic cross section of a part formed by SPF.
**FIGURE 4** is a schematic side elevation cross sectional view of a die and part manufactured by SPF.
**FIGURES 5A to 5F** show a cross section of a die and part in six consecutive stages of the SPF process of this invention.
**FIGURES 6A and 6B** show how the secondary sheet can entrap the blank after forming.
**FIGURE 7** is a schematic showing the axial and biaxial stresses around the cutout.
**FIGURE 8** compares thickness data at various locations on SPF parts made using prior art techniques and using the techniques of this invention.
**Figure 9A** shows an orthogonal projection of one-half of a SPF part.
**Figure 9B** shows a method for manipulating die surfaces to arrive at the size of a cutout of this invention.
**FIGURE 9C** illustrates a plan view of the blank after manipulating and projecting the die surfaces of Figure **9B**.

### Description of the Preferred Embodiment

One of the greatest challenges associated with Superplastic Forming is predicting material thinout and then achieving that thinout during part fabrication. The material thinout challenge is inherent to the SPF process and stems from varying material thickness across the part area after SPF. Engineering drawings typically call out a minimum allowed material thickness across the entire part or in specific regions of the part.

The reason that material does not thinout uniformly is that once the lid is closed on the SPF die, the periphery of the material is restrained such that the material is not allowed to "draw-in" from the edges. As a result, the material that will become the part area must be stretched from the material inside of the seal area.

During forming, the stretching of the material within the seal area progresses until the material eventually contacts the die surface. Upon contact, the material sticks to the die surface. The remaining material that has not yet contacted the die continues to stretch until it too contacts the die surface and sticks. Once the material is completely formed, the thinnest regions are generally those that are the last to form. These regions equate to the deepest areas of the die and radii, in particular spherical radii (corners).

Since material thinout is dependent on the die geometry, the die design is critical in achieving the proper material thinout. Of specific importance is the die "run-out", which is the die region outside the net part area. A correctly designed die will optimize the "run-out" configuration so that thinout is minimized in the part area and maximized in the "run-out" material.
Once the part area and "run-out" of the die have been machined and the rust SPF part is formed, there are only a few options for recourse if the part is too thin according to engineering drawing requirements. The two most common options are: (1) Start with a thicker gauge of blank material, (2) Preform the blank prior to forming it into the final part configuration.
The former option is the easier of the two options to implement and provides relatively quick results for thickness analysis. However, it is not a guarantee for achieving the correct minimum thickness since adding thickness to the starting blank does not equate to a sufficient thickness increase in the thinnest areas of the part. Furthermore, an increase in the starting material gauge adversely effects the part weight.

The latter option, designing a preform for the blank, carries a fair amount of risk. Designing a successful preform geometry potentially requires several iterations, an expensive and time consuming process. As with increasing the material gauge, preforming will not guarantee a successful part.

With this invention a third option becomes available for selectively increasing the material thickness in specific regions of the part. This option too, does not guarantee that the minimum material thinout will be attained. However, through a combination of increasing the starting gauge and utilizing this third option, the odds of attaining a successful part are significantly increased.

Depending on the part configuration, it is possible to minimize the material thinout by placing a strategically located cutout(s) in the starting blank. The typical applicable part configuration is one that has an area of the net trim that is internal to the part itself (i.e. a pocket or "bowl"). A simplified example would be a pan-shaped part that has the bottom of the pan cut away, resulting in a ring-shaped part.

Cutting out a hole(s) in the material allows for the hole(s) to enlarge as the material is stretched onto the tool surface. This enlarging takes the place of stretching and thinning the material if the holes were not present. The basic concept is that the hole enables more axial stretching of the material and minimizes the biaxial stretching (ref.Figure 5). The end result is minimized material thinout in the axially stretched material. The thinout in areas of the hole that are stretched biaxially is also minimized (relative to not using the cutout(s), but to a lesser extent than the axially stretched regions (ref. Figure 6 and Data Table I).

Since the SPF process uses gas pressure to form the material, it is imperative that the sheet being formed does not have any holes through it. This requirement is in direct opposition to the process of this invention. Subsequently, a second sheet of material that does not contain any cutout locations, is required to form the blank (material with the cutout(s). This second sheet is placed between the blank and the die lid and becomes the membrane which can be pressurized and formed onto the tool geometry. While forming, this secondary sheet also forms the blank with the cutout(s). Once the blank is fully formed (die surface is in intimate contact with the entire blank), the blank and secondary sheet are separated and the secondary sheet is discarded..

There are three critical factors that must be dealt with to successfully utilize the disclosed process. Those factors are: (1) Location of cutout(s) on the blank, (2) Shape and Size of the cutout(s) on the blank, and (3) Indexing the blank to the tool.
Cutout Location: The location of the cutout(s) is optimized when the periphery of the cutout(s) is located as close as possible to the net trim of the part after forming. Locating the cutout(s) as such will maximize the material thickness at the trim line.

Shape and Size of the Cutout(s): The cutout(s) shape and size are critical in that an undersized cutout will result in unnecessary thinout. Conversely, all oversized cutout will result in undercutting the trim line of the part. While both sizing and locating the cutout(s), caution must be taken so that the formed blank does not become entrapped by the secondary sheet during the separation of the two sheets (ref. Figure 6B).

There are several methods for determining the proper location and size of the cutout(s) on the blanks. Besides trial and error, a highly accurate "best guess" can be made utilizing a model of the die surface. Among the most easily manipulated mode is a Computer Aided Drafting (CAD) model. Once generated, the tool surfaces can be projected or rotated to one plane so that the trim line of the part can be seen on that plane - the equivalent of a forming blank (ref. Figure 9). This planar trim line defines a preliminary location, size, and shape of the cutout(s). The final size and shape of the cutout can then be obtained by applying a reduction factor to the preliminary size and shape.

Indexing the Blank to the Tool: Once the size, shape, and location of the cutout(s) have been determined, it is paramount that the blank be located to the die accurately. Without accurate, repeatable alignment, it is not possible to produce a consistent part. One method of locating the blank to the die is through the use of "pins" or "posts" that extend from the die sealing surface. Holes can then be cut into the blank and secondary sheet to correspond to the pins in the die.

### Description of Figures:

**Figure 5**: Illustrates the process steps for the Disclosed Invention Prior to Figure 5A, the region(s) of the blank that are to be cutout must be removed. The location, size and geometry of the cutout(s) is of critical importance for the successful forming of the part. In addition, it is also critical that the blank be indexed to the die surface so that the cutout area(s) form into the desired areas of the die.

**Figure 5A**: This figure illustrates the die, die lid, material blank and the secondary sheet. Once the die is heated to the forming temperature for the particular material alloy, the blank and secondary sheet are placed on the surface of the die. The location of the secondary sheet is between the die lid and the blank.

**Figure 5B**: The blank and secondary sheet are "sandwiched" between the die and lid by means of a force applied to the lid.

**Figure 5C**: As gas pressure is introduced to tile top side of the secondary sheet, the secondary sheet and blank are formed into the die cavity.

**Figure 5D**: Forming continues as the gas pressure is increased.

**Figure 5E**: Upon completion of the forming cycle, the blank is in full contact with the die surfaces.

**Figure 5F**: The gas pressure is vented and the lid is removed. The blank and secondary sheet are separated and removed from the die.

**Figure 6A**: This figure illustrates the result of correctly calculating and locating the cutout(s) on the blank. In this instance, the secondary sheet does not entrap the blank when the two are separated.

**Figure 6B**: This figure illustrates the potential problem of material entrapment caused by incorrectly calculating the size and location of the cutout(s) on the blank. In this instance after forming, the edge of the cutout(s) became located on a near-vertical surface, creating entrapment of the blank by the secondary sheet. This entrapment does not allow for separation of the blank and secondary sheet without cutting the two apart.

**Figure 7**: This figure illustrates tile types of stretching of the cutout periphery that take place during forming of the blank. Any straight line regions of the cutout periphery will undergo stretching in one direction (axial). Curved segments of the cutout will stretch in two directions (biaxial). In general, the axial stretching that takes place will result in less thinout than in the regions that are biaxially stretched.

**Figure 8**: This figure illustrates data obtained from fabricated test parts. All parts started with the same material thickness and were measured in the same locations. From the data it is possible to see that by cutting hole(s) in the blank, it is possible to achieve a 69% increase in as-formed material thickness, in comparison to parts formed without the invention process.

**Figure 9**: This figure illustrates how the basic geometry and location of the cutout(s) can be obtained. This key information be obtained through several methods. However, the easiest method is through the manipulation of Computer Aided Drafting (CAD) data of the die geometry. Use of such data is illustrated in this figure.

**Figure 9A**: This figure illustrates half of a symmetrical part. The dashed lines indicate surfaces of the die.

**Figure 9B**: This figure shows the axis about which the surfaces are rotated. Once the surfaces are rotated to the starting plane, a preliminary outline of the cutout can be determined. The edge of the surface rotated is determined by the net trim of the part.

## Claims

1. Method of forming a metal part by means of superplastic forming using pressurised gas, comprising the steps of:
- providing a blank sheet of metal, which is to be superplastically formed into the desired metal part;
- cutting out and removing portions of material of the sheet metal blank;
- locating a secondary sheet, which does not contain any cutout locations, in contact with said blank;
- locating the blank to a die;
- introducing pressurised gas into the die to force the blank there agains by contacting said secondary sheet, **characterized in that**
- the periphery of the blank is restrained from drawing in;
- the cutouts take the form of one or more holes, which holes are sized, shaped and located in the blank sheet of metal such as to decrease thinning of the blank during superplastic forming.

2. Method according to claim 1, wherein the secondary sheet does not contain any cut-outs in the form of holes.

3. Method according to claims 1 or 2, wherein the pressurized gas is introduced into the die, so that the secondary sheet is exposed thereto.

4. Method according to any of the preceding claims, wherein the cut out holes, is sized and located in the blank so that it increases in size during an appropriate cycle of superplastic forming.

5. Method according to any of the preceding claims, wherein the blank is aligned to the die, so that a periphery of the one or more cut out holes, falls into a predetermined tool surface of the die.

## Patentansprüche

1. Verfahren zum Formen eines Metallteils mittels superplastischem Formen unter Verwendung von Druckgas, umfassend die folgenden Schritte:
- Vorsehen eines Rohmetallblechs bzw. einer Rohmetallplatte, das bzw. die superplastisch zu dem gewünschten Metallteil geformt werden soll;
- Ausschneiden bzw. Heraustrennen und Entfernen von Teilen des Materials des Rohmetallblechs bzw. der Rohmetallplatte;
- Lokalisieren eines sekundären Blechs bzw. einer sekundären Platte, das bzw. die keinerlei Ausschnittsorte enthält, in Kontakt mit dem genannten Rohteil;
- Lokalisieren des Rohteils an bzw. in einer Form;
- Einführen von Druckgas in die Form, um das Rohteil durch Kontaktieren des sekundären Blechs bzw. der sekundären Platte dagegenzuforcieren bzw. zu drücken,
dadurch **gekennzeichnet**, daß
- der Umfang des Rohteils gegen ein Hineinziehen festgehalten bzw. arretiert wird;
- wobei die Ausschnitte die Form von einem oder mehreren Löchern annehmen, welche Löcher derart in dem Rohmetallblech bzw. der Rohmetallplatte bemessen, geformt und lokalisiert sind, daß das Verdünnen des Rohteils während des superplastischen Formens vermindert wird.

2. Verfahren gemäß Anspruch 1, worin das sekundäre Blech bzw. die sekundäre Platte keinerlei Ausschnitte in der Form von Löchern enthält.

3. Verfahren gemäß Anspruch 1 oder 2, worin das Druckgas so in die Form eingeführt wird, daß das sekundäre Blech bzw. die sekundäre Platte zu demselben hin freiliegt bzw. nach demselben exponiert ist.

4. Verfahren gemäß irgendeinem der vorhergehenden Ansprüche, worin die Ausschnittlocher bzw. das Ausschnittloch in dem Rohteil so bemessen und lokalisiert ist, daß es in der Größe während eines angemessenen Zyklus des superplastischen Formens zunimmt.

5. Verfahren gemäß irgendeinem der vorhergehenden Ansprüche, worin das Rohteil so zu der Form abgefluchtet ist, daß ein Umfang von dem einen oder mehreren Ausschnittlöchern in eine vorbestimmte Werkzeugoberfläche der Form fällt.

## Revendications

1. Procédé de formage d'une pièce métallique par formage à l'état superplastique à l'aide d'un gaz sous pression, comprenant les étapes suivantes :
la réalisation d'une feuille d'ébauche de métal destinée à subir le formage à l'état superplastique sous forme de la pièce métallique voulue,
la découpe et l'enlèvement de parties du matériau de l'ébauche de feuille métallique,
la disposition d'une feuille secondaire qui ne contient aucun emplacement de découpe, au contact de l'ébauche,
la disposition de l'ébauche sur un moule, et
l'introduction d'un gaz sous pression dans le moule afin que l'ébauche soit chassée contre lui, par contact avec la feuille secondaire,
caractérisé en ce que la périphérie de l'ébauche est retenue afin qu'elle ne puisse pas être tirée vers l'intérieur, et
les découpes ont la forme d'un ou plusieurs trous, les trous ayant des dimensions, configurations et emplacements dans la feuille métallique de l'ébauche tels que l'amincissement de l'ébauche est réduit pendant le formage à l'état superplastique.

2. Procédé selon la revendication 1, dans lequel la feuille secondaire ne contient aucune découpe sous forme de trous.

3. Procédé selon la revendication 1 ou 2, dans lequel le gaz sous pression est introduit dans le moule, si bien que la feuille secondaire est exposée à ce gaz.

4. Procédé selon l'une quelconque des revendications précédentes, dans lequel les trous des découpes ont des dimensions et emplacements dans l'ébauche tels que la dimension augmente au cours d'un cycle convenable de formage à l'état superplastique.

5. Procédé selon l'une quelconque des revendications précédentes, dans lequel l'ébauche est alignée sur le moule, si bien que la périphérie d'un ou plusieurs trous découpés se trouve sur une surface prédéterminée d'outil du moule.
